

# United States Patent [19]

Neidiffer et al.

[11] Patent Number: 4,959,105

[45] Date of Patent: Sep. 25, 1990

[54] ALUMINIUM CLEANING COMPOSITION AND PROCESS

[76] Inventors: **Fred Neidiffer**, P.O. Box 2497, Capistrano Beach, Calif. 92624; **Charles E. Fox; Patsy E. Fox**, both of Rte. #1, Box 87, Durant, Iowa 52747

[21] Appl. No.: 493,415

[22] Filed: Mar. 14, 1990

Related U.S. Application Data

[63] Continuation-in-part of Ser. No. 251,299, Sep. 30, 1988.

[51] Int. Cl.<sup>5</sup> ..... B08B 3/08

[52] U.S. Cl. ..... 134/3; 134/41; 252/79.4; 252/142; 252/174.12; 252/174.15

[58] Field of Search ..... 252/142, 174.12, 174.15, 252/79.4; 134/3, 41

[56] References Cited

U.S. PATENT DOCUMENTS

|           |         |                  |           |
|-----------|---------|------------------|-----------|
| 3,211,659 | 10/1965 | Pikaar et al.    | 1344/25.2 |
| 3,306,773 | 2/1967  | Laporte et al.   | 134/2     |
| 3,448,055 | 6/1969  | Mickelson et al. | 134/3     |
| 3,527,609 | 9/1970  | Vinso et al.     | 134/3     |
| 3,645,790 | 2/1972  | Burden et al.    | 134/3     |
| 4,049,467 | 9/1977  | Rubin            | 134/3     |
| 4,129,423 | 12/1978 | Rubin            | 134/3     |
| 4,256,602 | 3/1981  | McLaughlin, Jr.  | 252/142   |
| 4,264,418 | 4/1981  | Wood et al.      | 134/3     |
| 4,370,173 | 1/1983  | Dollman          | 134/3     |

|           |         |                 |            |
|-----------|---------|-----------------|------------|
| 4,435,223 | 3/1984  | Dollman         | 252/142    |
| 4,599,116 | 7/1986  | King et al.     | 134/3      |
| 4,713,119 | 12/1987 | Earhart et al.  | 134/3      |
| 4,728,456 | 3/1988  | Yamasoe et al.  | 134/3      |
| 4,806,259 | 2/1989  | Amjad           | 252/8.8    |
| 4,859,359 | 8/1989  | DeMatteo et al. | 252/174.15 |

Primary Examiner—Asok Pal

Attorney, Agent, or Firm—Gordon L. Peterson; Frank J. Uxa, Jr.

[57] ABSTRACT

A composition and process for cleaning an aluminum-containing article is disclosed. The process comprises contacting a debris-laden aluminum-containing article with a composition at conditions effective to do at least one of the following: (1) remove at least a portion of the debris from the aluminum-containing article and (2) condition at least a portion of the debris for removal from the aluminum-containing article. The composition comprises water; at least one polycarboxylic acid component selected from the group consisting of polycarboxylic acids, salts of polycarboxylic acids and mixtures thereof; at least one acidic component in an amount effective to increase the solubility of the polycarboxylic acid component in the composition; and at least one acid acting enzyme in an amount effective to at least facilitate the removal of debris from an aluminum-containing article contacted with the composition.

22 Claims, No Drawings

## ALUMINIUM CLEANING COMPOSITION AND PROCESS

### Related Application

This application is a continuation-in-part of application Ser. No. 251,299 filed Sept. 30, 1988, now pending.

### BACKGROUND OF THE INVENTION

This invention relates to a composition and process useful for cleaning aluminum-containing articles. More particularly, the invention relates to a composition and process for removing debris, e.g., smut, unwanted deposit material, soil and the like, from such articles, e.g., aluminum foodstuff or beverage containers or cans.

Aluminum-containing articles are often formed into shapes using lubricants to assist in the forming process. For example, one or more lubricants are often employed in the drawing and ironing of aluminum container bodies of the type used to package foodstuffs and beverages. The forming processing itself and/or the lubricant or lubricants employed produce debris, e.g., as noted above, on the article which interferes with the over-all appearance of the article. In certain instances, this debris is referred to as smut. In general, such smut or smut-like material includes aluminum and/or alumina fines and/or lubricant material and/or lubricant residue. Such debris should be removed to provide an aluminum-containing article which is visually pleasing and, more importantly, make the article suitable for use, e.g., as a foodstuff or beverage container.

Various compositions have been suggested for use in cleaning aluminum articles. For example, King, et al U.S. Pat. No. 4,599,116 discloses an aqueous alkaline (a pH of at least 10) cleaning composition containing an alkalinity agent present in an amount to achieve removal of aluminum fines, a complexing agent, and one or more surfactants. Preferred alkalinity agents include alkali metal hydroxides and alkali metal carbonates. Among the complexing agents are gluconic acid, citric acid, glucoheptonic acid, sodium triphosphate, EDTA, tartaric acid or the like, as well as the soluble and compatible salts thereof and mixtures thereof. The relatively strong alkalinity agents employed could harm, e.g., etch, the aluminum surface unless care was exercised to control the cleaning operation.

Dollman U.S. Pat. No. 4,370,173 discloses removing lubricating oils and aluminum fines from aluminum surfaces using an aqueous solution of sulfuric and hydrofluoric acids and an anionic surfactant. Michelson, et al U.S. Pat. No. 3,448,055 discloses removing smut from aluminum with an aqueous composition including nitric acid, sulfuric acid, hydrofluoric acid, phosphoric acid and a surfactant. Such solutions of strong acids are effective to clean the aluminum surfaces, but also tend to etch the surface as well. Such etching is undesirable.

Earhart U.S. Pat. No. 4,713,119 discloses removing alkali metal aluminum silicate deposits from chemical processing equipment by alternating treatments with acidic and basic solutions. The acidic solution contains sulfuric acid, sodium bisulfate, tartaric acid or phosphoric acid. This patent does not disclose cleaning aluminum-containing surfaces nor that the acidic solution includes a surfactant.

Wood, et al U.S. Pat. No. 4,264,418 discloses removing oxide film from metals or alloys containing iron, nickel, copper, beryllium, chromium, gold, zinc, lead,

or tin with a composition containing gluconic acid or its alkali metal salts, citric acid or its alkali metal salts, or tartaric acid or its alkali metal salts and, preferably, a non-ionic surfactant. Aluminum-containing articles are not disclosed. Further, no "strong" acid is included in the composition.

Laporte, et al U.S. Pat. No. 3,306,773 discloses treating sintered aluminum parts with an aqueous alkaline solution before putting such parts into heat transfer surface. Pikaar U.S. Pat. No. 3,211,659 discloses acids, such as acetic acid, EDTA, citric acid, tartaric acid, gluconic acid, glyceric acid, malic acid, glycolic acid, saccharic acid, phosphoric acid, and benzoic acid for cleaning egg shells. Vinso U.S. Pat. No. 3,527,609 discloses the use of tartaric acid salts among salts of many polycarboxylic acids for use in cleaning cooling water systems. Rubin U.S. Pat. Nos. 4,049,467 and 4,129,423 disclose removing manganese derived discolorations from hard surfaces by use of either dihydroxy maleic acid, dihydroxy tartaric acid, their alkali metal salts, or mixtures thereof. None of these references is concerned with relatively heavy duty cleaning of, e.g., smut removal from, aluminum surfaces.

Yamasoe et al U.S. Pat. No. 4,728,456 discloses an aluminum surface cleaner which is an aqueous highly acidic solution containing sulfuric acid and/or nitric acid, ferric ions, but no chromium or fluoride ions. Yamasoe et al discloses that the etching of the aluminum by the sulfuric acid or nitric acid is promoted by the ferric ions. Also, Yamasoe et al discloses that chelating agents, such as citric acid and tartaric acid, can be included to accelerate the aluminum etching rate.

### SUMMARY OF THE INVENTION

A new composition and process for cleaning debris, in particular smut, from the surface of an aluminum-containing article had been discovered. This invention provides very effective and efficient cleaning, e.g., removal of debris, with little or no substantial adverse effect on, e.g., etching of, the surface being cleaned. Thus, although the present composition includes at least one relatively strong acid, e.g., sulfuric acid, such acid often acts as a solubilizing agent rather than as the primary cleaning agent in removing debris from the aluminum-containing surface. In short, the present composition is specifically designed to clean, and not to etch, aluminum-containing surfaces.

In one broad aspect, the present invention involves a process for cleaning debris from the surface of an aluminum-containing article. This process comprises contacting a debris-laden aluminum-containing article with a composition comprising water, at least one polycarboxylic acid and/or at least one salt thereof, at least one acidic component in an amount effective to increase the water solubility of the polycarboxylic acid and/or salt thereof, and at least one acid acting enzyme in an amount effective to at least facilitate the removal of debris from the surface of the aluminum-containing article; and recovering the aluminum-containing article having at least a portion of the debris removed therefrom. The contacting occurs at conditions effective to do at least one of the following: remove at least a portion of the debris from the aluminum-containing article and condition at least a portion of the debris for removal from the aluminum-containing article. The composition may also include, or all or a portion of the enzyme may be replaced by, at least one acid compatible siloxane

component in an amount effective to at least facilitate the removal of at least a portion of the debris from the aluminum-containing article. Further, the composition preferably includes at least one surface active component, i.e., surfactant.

The use of the present- enzymes and/or the siloxane components has been found to provide enhanced aluminum cleaning without substantial adverse effects on, e.g., etching of, the surface being cleaned. The effective and beneficial use of enzymes in aluminum cleaning, especially in the relatively highly acidic present compositions, is unexpected. One particularly surprising feature of the present invention is the inclusion of acid-compatible siloxane components and the beneficial aluminum cleaning resulting therefrom. For example, other materials of the same general class, such as silanes, have not been found to provide such enhanced aluminum cleaning.

#### DETAILED DESCRIPTION OF THE INVENTION

The present compositions comprise water, at least polycarboxylic acid and/or salts thereof, at least one additional acidic component, and at least one acid acting enzyme and/or at least one acid compatible siloxane component. The water often, and preferably, acts as a carrier for the other components of the composition. Water preferably comprises a major amount, i.e., at least about 50%, by volume, and more preferably at least about 70% by volume, of the composition used to treat the aluminum-containing article. In certain instances, it is desirable to prepare the present compositions in the form of one or more concentrates, with reduced amounts of water. The use of such concentrate or concentrates reduces the cost of transporting the present composition to the cleaning site. Thus, the present compositions can be formulated at the cleaning site simply by combining the desired amounts of concentrate or concentrates and water.

In a particularly useful embodiment, two concentrates are prepared. One concentrate includes the polycarboxylic acid and/or salts thereof and the additional acidic component in water, while the other concentrate includes the enzymes and/or the siloxane component, preferably together with one or more surfactants. This is particularly useful in situations where it is difficult or impossible to include all the presently useful components in one concentrate which is substantially homogeneous, e.g., clear. For example, if the surfactant mixture includes a substantially hydrocarbonaceous component, e.g., a mineral oil component, such component has only limited water solubility and does not form a homogeneous concentrate with the other components of the present composition. Also, the enzyme and/or siloxane component may not form a completely homogenous concentrate with the acid components. In this instance, the enzyme and/or siloxane component and/or surfactant are best employed as a separate concentrate which is combined with the other components at the cleaning site when the full amount of water is present.

The acid acting enzymes included in the present invention are present in an amount effective to at least facilitate the removal of debris from an aluminum-containing article contacted with the enzyme-containing composition. One enzyme or a combination of enzymes may be employed. Acid acting enzyme means an enzyme which is effective or active in an acidic environment, in particular in the present aluminum cleaning

compositions. The exact nature of the enzymatic action is not fully understood, although aluminum cleaning benefits are obtained provided that the enzyme or enzymes are effective in the relatively highly acidic compositions of the present invention. Such compositions preferably have a pH in the range of about 0.5 to about 3, more preferably about 0.8 to about 2. Without wishing to limit the scope of the present invention to any particular theory of operation, it is believed that the present acid acting enzyme or enzymes act on at least a portion of the debris on the aluminum-containing article to change its character and thereby render it more easily removable from the surface of the aluminum-containing article.

Examples of suitable acid acting enzymes include: enzyme derived from the fermentation of *B. licheniformis*, such as that sold by Genecor under the trademark Rhozyme P-64; enzyme extracted from pineapple stems, such as that sold by Miles under the tradename Bromelain 1:10; and enzyme derived from the fermentation of *Aspergillus niger*, such as that sold by Miles under the trademark Milezyme APF-2000. The amount of enzyme in the present compositions is relatively minor. The enzyme is preferably present, if at all, in an amount in the range of about 0.0001% to about 0.5% by weight of the total composition. Excessive amounts of enzyme are to be avoided in view of the relatively high cost of such materials. Enzyme preparations which are commercially sold often include materials other than the active enzyme, and may include as little as about 10% by weight, or even less, of the active enzyme. The amounts of enzyme noted in this paragraph refer to the active enzyme.

The siloxane components included in the present invention are present in an amount effective to at least facilitate the removal of debris from an aluminum-containing article contacted with the siloxane component-containing composition. Acid compatible siloxane component means a siloxane component which is dispersible, preferably soluble, in the present composition. The present siloxane components are polymeric materials having the characteristic siloxane structure included in the polymer, e.g., the backbone of the polymer. Such polymeric materials may, and preferably do, include one or more substituents, e.g., on the siloxane repeating unit of the polymer. Such substituents may include, for example, carbon, hydrogen, oxygen and nitrogen atoms. The siloxane component is preferably selected to minimize, and more preferably to substantially avoid, chemical reaction, e.g., acid/base reaction, between the siloxane component and the acid or acids of the present composition. Thus, it is preferred that the siloxane component preferably be substantially free of reactive amino groups. Also, it is preferred that the siloxane component be substantially free of sulfur, in particular mercapto groups. Such mercapto-containing siloxane components have been found to not provide aluminum cleaning benefits to the extent exhibited by other siloxane components.

It is particularly surprising that the present siloxane components provide beneficial aluminum cleaning since other silicone polymers, such as the silanes, are much less effective, and even substantially ineffective, in providing enhanced aluminum cleaning. Both the siloxane components and the silane components are effective defoamers in the present compositions. This fact makes the aluminum cleaning benefits achieved with the siloxane components all the more unexpected.

Examples of suitable siloxane components include: gamma-amino propyl trimethyl siloxane, such as that sold by PCR, Incorporated under the trademark Prosil 220; and gamma-methoxy-acryloxy propyl trimethyl siloxane, such as that sold by PCR, Incorporated under the trademark Prosil 248 and that sold by Dow Corning under the trademark Z-6030. The amount of siloxane component in the present compositions is preferably relatively minor. The siloxane component is relatively present in an amount in the range of about 0.0001% to about 0.5%, more preferably about 0.0005% to about 0.2%, by weight of the total composition. Excessive amounts of the siloxane component are to be avoided in view of the relatively high cost of such materials.

The polycarboxylic acid component, i.e., one or more polycarboxylic acid and/or salts thereof, useful in the present invention provide substantial advantages. The polycarboxylic acid component is preferably present in an amount effective to at least facilitate at least one of the following: (1) remove at least a portion of the debris from the aluminum-containing article; and (2) condition at least a portion of the debris for removal from the aluminum-containing article. Polycarboxylic acid refers to a carboxylic acid having more than one functional hydroxyl group, preferably two or three functional hydroxyl groups. The polycarboxylic acid component preferably includes 2 to about 10 carbon atoms per molecule. Without wishing to limit the scope of the invention to any particular theory of operation, it is believed that this polycarboxylic acid component plays a substantial role or roles in removing debris from the aluminum-containing article. For example, in many instances the debris to be removed includes organic material, such as residues from lubricants, e.g., containing fatty acids, used in forming or shaping the aluminum-containing article. It is believed that the polycarboxylic acids and/or salts thereof are particularly effective in attacking this organic material, especially to reduce the ability of such organic material to adhere or cling to the aluminum-containing surface. By compromising this organic material, this polycarboxylic acids component is also believed to act to facilitate removing aluminum particles (which are often a part of the debris) from the surface. While the polycarboxylic acid component provides effective debris cleaning/conditioning action, this component is insufficiently strong or aggressive to attack the aluminum-containing surface itself. Thus, the debris is removed and the aluminum-containing surface remains substantially unaffected, e.g., unetched.

Among the suitable polycarboxylic acids are: citric acid, tartaric acid, saccharic acid, maleic acid, oxalic acid, malonic acid, succinic acid, glutaric acid, adipic acid, pimelic acid, suberic acid, azelaic acid, sebacic acid, diglycolic acid, phthalic acid and the like. The preferred polycarboxylic acid is tartaric acid, in particular the racemic form of tartaric acid.

Any suitable source of polycarboxylic acid and/or salts thereof may be employed. If a salt is used, it is preferred that the salt be an ammonium salt, an alkali metal salt, an alkaline earth metal salt or mixtures thereof, more preferably an alkali metal salt. A particularly useful source of tartaric acid component is cream of tartar or potassium hydrogen tartrate. The polycarboxylic acid component is present in an amount effective to function as described herein. Preferably, the polycarboxylic acid component is present in the composition in an amount in the range of about 0.1% to about

20%, more preferably about 2% to about 15%, by weight, calculated as the polycarboxylic acid.

Polycarboxylic acids and/or salts thereof often have relatively limited water solubility. Thus, the presently useful additional acidic component is present in an amount effective to increase the water solubility of such polycarboxylic acid component. Such additional acidic component preferably is stronger, i.e., has a larger dissociation constant, than the polycarboxylic acid being employed. Examples of suitable acidic components include sulfuric acid, phosphoric acid, hydrochloric acid, hydrofluoric acid, nitric acid, mixtures thereof and the like, with sulfuric acid, phosphoric acid and mixtures thereof being preferred.

Care should be exercised to avoid having excessive amounts of such additional acidic components present. Such excessive amounts of acidic components may interact with the aluminum-containing article and cause damage, e.g., etching, of the surface being cleaned. However, it should be noted that in a particularly useful embodiment of the present invention, the acidic component is present in an amount effective to solubilize aluminum fines which may be part of the debris to be removed from the aluminum-containing article. The amount of acidic component included in the present composition may vary over a wide range and depend on many factors, for example, on the particular acid or acids being employed, on the particular debris to be removed, on the chemical make-up of the present composition and on the particular cleaning application involved. In certain embodiments it is preferred to include sufficient acidic component to maintain a pH in the range of about 0.5 to about 3, more preferably about 0.8 to about 2, during the contacting step.

The present compositions preferably include at least one surface active component or surfactant. In general, such surface active component or components act to increase or enhance the effectiveness of the composition, e.g., as an aluminum cleaner. However, it is not all together clear how such component or components function in the present invention. Without wishing to limit the invention to any particular theory of operation, it is believed that the surface active component or components act to do at least one of the following: (1) assist in removing the organic portion of the debris from the surface of the aluminum-containing article; (2) aid in maintaining the homogeneity of the composition during use; and (3) aid in preventing or inhibiting redeposition of the removed debris onto the surface of the aluminum-containing article.

Any suitable surface active component or combination of such components may be employed in the present compositions. Such component is preferably non-ionic or anionic, with anionic surfactants being particularly preferred. The surface active component preferably has a Hydrophile-Lipophile Balance (HLB ratio), i.e., the balance of the size and strength of the hydrophilic (water-loving or polar) and lipophilic (oil-loving or non-polar) groups of the molecules, of at least about 12, more preferably in the range of about 12 to about 15. For further information regarding the determination of the HLB number of surfactants and emulsifying agents, reference is made to a publication entitled "The Atlas HLB System", Third Edition, 1963, by Atlas Chemical Industries, Inc.

Surfactants suitable for use in the practice of the present invention include, for example, those having hydrophobic groups comprising alkyl phenols, linear

alcohols, branched-chain alcohols, secondary alcohols, propylene oxide/propylene glycol condensates and the like; hydrophilic groups such as ethylene oxide, ethylene oxide/ethylene glycol condensates and the like, and may further contain capping groups such as propylene oxide, chloride, benzyl chloride, amines and the like.

Specific examples of useful surfactants include free acids of complex organic phosphate esters (e.g., Gafac RP 170 from GAF Corporation); block polymers of propylene oxide and ethylene oxide (e.g., Pluonic L-61 from BASF Wyandotte, Inc.); ethoxylates of secondary alcohols containing about 11 to about 15 carbon atoms per molecule (e.g., Tergital 15-S-3 from Union Carbide Corporation); blends of linear alkyl sulfates and ethoxylates of secondary alcohols (as noted above); blends of anionic surfactants including ammonium laurel sulfate, lauramide diethanol amine, sodium laurel sarcosinate, and propyl ethyl diammonium ethosulfate; sodium linear alkyl sulfonate (e.g., Darvan No.1 from R. T. Vanderbilt Company, Inc.); and the like. A particularly useful component, especially in combination with one or more other surface active components, comprises a mixture of one or more surfactants, especially anionic surfactants, such as dodecyl benzene sulfonic acid, together with at least one substantially hydrocarbonaceous material, such as paraffinic mineral oil. This mixture may also include water. The substantially hydrocarbonaceous material is believed to be particularly effective in removing organic debris from the aluminum-containing article. A specific example of such particularly useful component is Wax Emulsion M from Northwest Chemical Co. An aqueous material including dodecyl benzene sulfonic acid without paraffinic mineral oil, such as that sold by Northwest Chemical Co. under the trademark Northwest 3867, is also particularly useful.

The surfactant or combination of surfactants can be employed in the present compositions in concentrations which are effective to provide enhanced cleaning, i.e., relative to cleaning with a composition having no such surfactant or surfactants. Preferably, the surfactant or combination of surfactants are employed at concentrations in the range of about 0.01% to about 2%, more preferably about 0.05% to about 1%, by weight of the composition.

One or more coupling agents, e.g., conventional coupling agents such as butyl cellosolve, isopropyl alcohol and the like, may be included in the present compositions to provide increased homogeneity to the present composition (or to the concentrate from which the present composition is derived).

In accordance with the present invention, the present composition is applied to the debris-laden aluminum-containing article at comparatively low to moderate temperatures. Preferred composition/aluminum-containing article contacting temperatures are in the range of about 60° F. to about 150° F. with lower temperatures, e.g., about 60° F. to about 110° F. being particularly useful to provide effective cleaning while having no substantial adverse impact on, e.g., etching of, the aluminum-containing article. The contacting of the aluminum-containing articles to be cleaned can be effected by flooding, immersing, dipping, spraying and the like.

The aluminum-containing article may be subjected to a rinse step, e.g., with liquid water, to obtain removal, or more complete removal, of the debris. This rinse can be effected by flooding, immersing, dipping, spraying

and the like of the article with or in the rinse material, e.g., at the temperatures noted above. In any event, after contact with the present composition, and the rinse step if desired or necessary, the aluminum-containing article is recovered and has a reduced amount, i.e., relative to the original debris-laden article, of debris on its surface.

The following non-limiting examples illustrate certain aspects of the present invention.

#### EXAMPLE 1

The following composition has prepared by blending together the various components with stirring:

|                                                       | Wt %   |
|-------------------------------------------------------|--------|
| Water                                                 | 92.5   |
| Sulfuric Acid (25% by weight in water)                | 0.7    |
| Cream of Tartar (potassium bitartrate) <sup>(1)</sup> | 6.5    |
| Surfactant I <sup>(2)</sup>                           | 0.07   |
| Surfactant II <sup>(3)</sup>                          | 0.07   |
| Surfactant III <sup>(4)</sup>                         | 0.03   |
| Surfactant IV <sup>(5)</sup>                          | 0.13   |
|                                                       | 100.00 |

<sup>(1)</sup>This material includes tartaric acid functionality in the racemic form.

<sup>(2)</sup>A commercially available anionic material including a free acid of a complex organic phosphate ester.

<sup>(3)</sup>A commercially available nonionic material including block copolymers of propylene oxide and ethylene oxide.

<sup>(4)</sup>A commercially available nonionic material including ethoxylates of secondary alcohols containing about 11 to about 15 carbon atoms per molecule.

<sup>(5)</sup>A commercially available blend of anionic and nonionic surfactants, believed to be linear alkyl sulfates together with ethoxylates of secondary alcohols as noted in (4) above.

This composition was tested as an aluminum cleaner by immersing a formed aluminum beverage can in the composition for about 15 minutes, at ambient temperature, i.e., about 70° F. to about 75° F., unless otherwise noted. This formed aluminum beverage can was contaminated by smut, a mixture including aluminum and alumina fines and fatty acid residues from the lubricant used in forming the can. This immersion or washing step was followed by a rinsing step in which the can was removed from the composition and placed in a bath of water, for about 15 minutes at ambient temperatures and then removed. Visual observation was used to determine the effectiveness of the composition as an aluminum cleaner.

The above-noted composition provided some smut removal during the washing step. Substantially all of the remaining smut was removed during the rinsing step so that a clean aluminum beverage can resulted. Moreover, except for smut removal, the can was substantially unaffected by the treatment. For example, no evidence of aluminum etching was observed. Such etching is undesirable and has often occurred in the past with cleaning compositions including relatively large concentrations of strong acids, such as sulfuric acid, hydrofluoric acid and the like.

#### EXAMPLE 2

Example 1 was repeated except that the final composition included an additional 4.4% by weight of the levo form of tartaric acid. The cleaning results obtained with this composition were similar to the results obtained in Example 1. For example, substantially no additional smut removal was obtained during the washing step. Thus, it surprisingly appears that the racemic form of

tartaric acid is more effective than the levo form in the present invention.

In both Example 1 and 2, heating the compositions had substantially no effect on the aluminum cleaning results.

### EXAMPLE 3 TO 14

A series of compositions were prepared by blending together various components. Each of these compositions included the following:

|                                        | Wt. gms. |
|----------------------------------------|----------|
| Water                                  | 300      |
| Sulfuric Acid (25% by weight in water) | 1.5      |
| Surfactant V <sup>(6)</sup>            | 0.8      |
| Surfactant I                           | 0.3      |
| Surfactant III                         | 0.1      |
| Butyl carbitol (coupling agent)        | 0.3      |

<sup>(6)</sup>Similar to Surfactant II.

Additional components were included in the various compositions, as indicated below. Each of these compositions was used as an aluminum beverage can cleaner as outlined in Example 1.

| Test | Example <sup>(7)</sup> | Additional Component, gms., (Wt %)                                                    | Comments on Cleaning                                                                                                                                  |
|------|------------------------|---------------------------------------------------------------------------------------|-------------------------------------------------------------------------------------------------------------------------------------------------------|
| 3    |                        | Formic acid 1.2 gms.(0.4%)                                                            | No effective cleaning                                                                                                                                 |
| 4    |                        | Acetic acid 1.7 gms.(0.6%)                                                            | No effective cleaning.                                                                                                                                |
| 5    |                        | Sulfuric acid (25% by weight in water) 25 gms. (7.6%)                                 | Cleaning did not work well.                                                                                                                           |
| 6    |                        | Surfactant IV 3 gms.(1.0%)                                                            | Cleaning did not work well.                                                                                                                           |
| 7    |                        | Sulfuric acid (25% by weight in water) 25 gms. (7.6%) plus Surfactant IV 3 gms (0.9%) | Cleaning worked well. Potential for harmful aluminum etching was present because of relatively high concentration of H <sub>2</sub> SO <sub>4</sub> . |
| 8    |                        | Propionic acid 10 gms. (3.2%)                                                         | No effective cleaning                                                                                                                                 |
| 9    |                        | Butyric acid 10 gms.(3.2%)                                                            | Not all butyric acid soluble, substantial cleaning observed.                                                                                          |
| 10   |                        | Crotonic acid 10 gms.(3.2%)                                                           | Only 3 gms. of crotonic acid soluble, no effective cleaning                                                                                           |
| 11   |                        | Hydroxy acetic acid 10 gms. (3.2%)                                                    | Does not form clear solution, no effective cleaning.                                                                                                  |
| 12   |                        | Sodium ethylene diamine tetra acetate 10 gms.(3.2%)                                   | Not soluble in composition, did attack smut when crystals dissolved during rinsing.                                                                   |
| 13   |                        | Ascorbic acid 10 gms.(3.2%)                                                           | Substantial cleaning observed, not as effective as with cream of tartar composition.                                                                  |
| 14   |                        | Citric acid 10 gms.(3.2%)                                                             | No effective cleaning                                                                                                                                 |

<sup>(7)</sup>As a base line, the composition described above, with no additional components, was tested as an aluminum beverage can cleaner. No effective cleaning was observed. These results indicate that various other additive materials do not provide the combination of benefits, e.g., effective aluminum cleaning with little or no risk of aluminum damage, achieved by the present composition and method. Further, it should be noted that a cleaning composition which precipitates one of its components can be detrimental to the high speed cleaning operations often used in producing aluminum articles, e.g., beverage cans.

As a base line, the composition described above, with no additional components, was tested as an aluminum beverage can cleaner. No effective cleaning was ob-

served. These results indicate that various other additive materials do not provide the combination of benefits, e.g., effective aluminum cleaning with little or no risk of aluminum damage, achieved by the present composition and method. Further, it should be noted that a cleaning composition which precipitates one of its components can be detrimental to the high speed cleaning operations often used in producing aluminum articles, e.g., beverage cans.

### EXAMPLES 15 TO 18

The following composition, Example 15, was prepared by blending together the following components:

|                                        | Wt., gms. |
|----------------------------------------|-----------|
| Water                                  | —         |
| Sulfuric acid (25% by weight in water) | 37        |
| Cream of Tartar                        | 20        |
| Surfactant V                           | 1.1       |
| Surfactant I                           | 0.4       |
| Surfactant III                         | 0.1       |
| Surfactant IV                          | 2         |
| Butyl cellosolve                       | 5         |
| Isopropyl alcohol                      | 5         |
| Commercially available defoaming agent | 0.03      |

In Example 16, a composition as set forth above was similarly prepared except that the Surfactant IV was replaced by a commercially available blend of anionic surfactants (Surfactant VI) which included ammonium lauryl sulfate; lauramide diethanol amine; sodium lauryl sarcosinate; and isostearamide propyl ethyl diammonium ethosulfate.

In Example 17, a composition as set forth in Example 15 was similarly prepared except that 4 gms. of a commercially available mixture of water, dodecyl benzene sulfonic acid (anionic) and paraffinic mineral oil (Surfactant VII) was included.

In Example 18, a composition as set forth in Example 15 was similarly prepared except that 4 gms. of a commercially available anionic material including sodium linear alkyl sulfonate (Surfactant VIII) was included.

Each of the above-noted compositions was tested as an aluminum beverage can cleaner as outlined in Example 1. Results of these tests are summarized as follows:

| Example | Comments on Cleaning Test                                                                                                                                                  |
|---------|----------------------------------------------------------------------------------------------------------------------------------------------------------------------------|
| 15      | This composition provided effective cleaning. Without the water component, the formula is an unstable emulsion and therefore may present handling problems.                |
| 16      | This composition provided effective cleaning. The dispersed smut in the composition (after washing) precipitated out of the composition.                                   |
| 17      | This composition provided a very clean can. Without the water component, Surfactant VII was not stable, i.e., did not form a homogenous mixture with the other components. |
| 18      | This composition did not clean as effectively as did the composition of Example 17.                                                                                        |

-continued

| Example | Comments on Cleaning Test                                         |
|---------|-------------------------------------------------------------------|
|         | Thus, the paraffinic mineral oil may play a role in smut removal. |

## EXAMPLES 19 TO 22

A base composition as prepared by blending together 10 the various components with stirring:

|                                        | Wt., Gms. |
|----------------------------------------|-----------|
| Sulfuric acid (25% by weight in water) | 91        |
| Cream of tartar                        | 49        |
| Surfactant VIII                        | 4         |
| Surfactant IV                          | 3         |
| Commercially available defoaming agent | 0.3       |

In addition, a series of four (4) other surfactants were included, one in each of four (4) samples of the above-noted composition. These other surfactants were included in an attempt to produce a stable or clear concentrate which provided effective aluminum cleaning.

In Example 19, a commercially available material including sodium n-hexadecyl diphenyloxide disulfonate (Surfactant IX) was used. In Example 20, a commercially available material including octyl phenoxy polyethoxy ethanol (Surfactant X) was used. In Example 21, a commercially available material including nonyl phenoxy poly(ethylenoxy) ethanol (Surfactant XI) was used. In Example 22, a commercially available material including aliphatic polyalkoxylates (Surfactant XII) was used.

Each of these concentrates was allowed to stand quiet for a period of time and then observed. Results of these observations are summarized as follows:

| Example | Observations                                                                                                                                                                                                                                      |
|---------|---------------------------------------------------------------------------------------------------------------------------------------------------------------------------------------------------------------------------------------------------|
| 19      | This concentrate was clear. However, when it was combined with additional water and used to clean aluminum beverage cans, as set for in Example 1, its cleaning performance was poor relative to other compositions derived from cream of tartar. |
| 20      | Concentrate was cloudy and separated.                                                                                                                                                                                                             |
| 21      | Concentrate was very cloudy.                                                                                                                                                                                                                      |
| 22      | Concentrate was cloudy and separated.                                                                                                                                                                                                             |

These results indicate that if all the components, other than a substantial portion of the water, are to be included in a single mixture it may be important to effectively stir the concentrate before combining it with water for aluminum cleaning. In addition, these results also indicate that if a clear composition is deemed necessary, e.g. for marketing purposes, it may be necessary to provide the concentrated form of the present composition as two or more concentrates.

## EXAMPLE 23

Two separate concentrates were prepared blending together the following components:

Wt %

|   | Concentrate A                          | Concentrate B                          | Wt % |
|---|----------------------------------------|----------------------------------------|------|
| 5 | Cream of tartar                        | Surfactant VII                         | 35.3 |
|   | Sulfuric acid (25% by weight in water) | Surfactant IV                          | 64.7 |
|   | Density 1.39 gms/ml.                   | Commercially available defoaming agent | 72   |
|   |                                        |                                        | 20   |
|   |                                        |                                        | 1    |
|   |                                        | Density 0.93 gms/ml.                   |      |

15 Each of these concentrates was substantially clear. A cleaning composition was prepared by combining Concentrate A, at a rate of 9 fluid oz. per gallon, and Concentrate B, at a rate of 1.2 fluid oz. per gallon, with water. The resulting clear composition was tested as an aluminum beverage can cleaner as set forth in Example 1. All of the smut was removed from the can, and no foaming problems were encountered.

25 These results demonstrate one alternative to using a single non-homogeneous concentrate. Thus, the cleaner can be manufactured as two, or more, substantially clear (homogeneous) concentrates, which are then shipped to the cleaning site, combined with water and made ready for use as an aluminum cleaner.

30 While this invention has been described with respect to various specific examples and embodiments, it is to be understood that the invention is not limited thereto and that it can be variously practiced within the scope of the 35 following claims.

## EXAMPLES 24 TO 29

The following acid composition was prepared by blending together the following components:

|    | Wt. %                                    |
|----|------------------------------------------|
| 45 | Sulfuric Acid (98% by weight in water)   |
|    | Sulfuric acid (25% by weight in water)   |
|    | Phosphoric acid (85% by weight in water) |
|    | Creme of tartar                          |

50 A series of six (6) enzymes were selected for testing to determine the effect of the enzyme in aluminum cleaning. Each enzyme was included in a composition which had the following make-up:

|                                |        |
|--------------------------------|--------|
| Water                          | 300 g. |
| Base Acid Composition          | 23 ml. |
| Surfactant XIII <sup>(8)</sup> | 0.5 g. |
| Enzyme <sup>(9)</sup>          | 0.5 g. |

60 <sup>(8)</sup>A commercially available amonic surfactant including a mixture of water and dodecyl benzene sulfonic acid.

<sup>(9)</sup>Each enzyme was included as, and the weight based on, the commercially available enzyme-containing preparation.

65 Each composition was tested as an aluminum cleaner in accordance with the test procedure outlined in Example 1.

Results of these tests were as follows:

| Example | Enzyme            | Cleanliness Rating <sup>(16)</sup> | Compatibility Rating <sup>(17)</sup> |
|---------|-------------------|------------------------------------|--------------------------------------|
| 24      | A <sup>(10)</sup> | Excellent                          | Excellent                            |
| 25      | B <sup>(11)</sup> | Good                               | Good                                 |
| 26      | C <sup>(12)</sup> | Good                               | Poor                                 |
| 27      | D <sup>(13)</sup> | Fair                               | Poor                                 |
| 28      | E <sup>(14)</sup> | Poor                               | Poor                                 |
| 29      | F <sup>(15)</sup> | Poor                               | Fair                                 |

<sup>(10)</sup>Enzyme derived from the fermentation of *B. licheniformis*. Claimed to be more than 40% active at pH 3.0. Sold by Genecor under the trademark Rhozyme P-64.

<sup>(11)</sup>Enzyme extracted from pineapple stems. Claimed to be effective at pH 3.0. Sold by Miles under the trademark Bromelain 1:10.

<sup>(12)</sup>Enzyme derived from fermentation of *Aspergillus niger*. 100% active at pH 3.0. Sold by Miles under the trademark Milezyme APF-2000.

<sup>(13)</sup>Enzyme derived from fermentation of *B. subtilis*. Claimed to be inactive at pH 3.0. Sold by Genecor under the trademark Rhozyme P-53.

<sup>(14)</sup>Enzyme extracted from *Carica papaya* fruit. Is ineffective below pH 3.0. Sold by Miles under the trademark Papain 16000.

<sup>(15)</sup>Enzyme is an alkaline protease-serine endopeptidase. Is effective above pH 7.0. Sold by Gist-Brocades under the trademark Maxatase. LS-400,000.

<sup>(16)</sup>Cleanliness rating was based on degree of soil removal from the can into the composition as indicated by the darkening of the composition and by the lack of aluminum fines or smut left on the can. "Excellent" was taken as complete removal of fines and smut from the can, while "poor" was taken to be little or no darkening of the composition and little or no removal of fines and smut from the can.

<sup>(17)</sup>Compatibility rating was based on the ability of the enzyme to mix with the anionic surfactant and/or acid composition and form a clear solution or a stable emulsion.

These results demonstrate that acid active enzymes are effective to enhance aluminum cleaning. Also, care is to be exercised in selecting the acid active enzyme for use in the present invention if the materials from which the final cleaning compositions are derived, e.g., by blending with water, are to be clear solutions and/or stable emulsions.

#### EXAMPLES 30 TO 34

A series of (5) compositions were prepared by blending the following components together:

#### EXAMPLE E

|                                                                | 30    | 31    | 32    | 33    | 34    |
|----------------------------------------------------------------|-------|-------|-------|-------|-------|
| Water                                                          | 300 g | 300 g | 300 g | 300 g | 600 g |
| Acid Composition<br>(as in Examples 24-29)                     | 23 ml | 23 ml | 23 ml | 23 ml | 23 ml |
| Enzyme A                                                       | 0.5 g |       |       |       |       |
| Surfactant XIII                                                |       | 0.5 g |       |       |       |
| Lithium salt of<br>Fluoroalkylthionyl acid                     |       |       | 0.1 g |       |       |
| Commercially available<br>food grade silicon-based<br>defoamer |       |       |       | 0.2 g | 0.2 g |

Each composition was tested as an aluminum cleaner in accordance with the procedure outlined in Example 1. In addition, the foaming characteristics of the composition were observed.

5 Results of these tests were as follows:

| Example | Cleanliness Rating | Foaming Characteristics |
|---------|--------------------|-------------------------|
| 30      | Fair               | No foam                 |
| 31      | Excellent          | Very high foam          |
| 32      | Excellent          | High foam               |
| 33      | Excellent          | Low foam                |
| 34      | Good               | Low foam                |

15 These results indicate that a silicon-based defoamer is useful in the present compositions to reduce foam. In addition, such silicon-based material may have a beneficial effect on the aluminum-cleaning ability of the composition.

#### EXAMPLES 35 TO 43

A series of compositions was prepared and tested as aluminum cleaners in accordance with the procedure outlined in Example 1 to illustrate the beneficial effect on aluminum cleaning of certain silicon-based materials.

Each of these compositions was prepared by adding 0.5 gm. of the specific silicon-based material being tested to 23 ml of the acid composition described in Examples 24 to 29. At this point, the mixture was observed for compatibility. After this observation, the mixture was combined with 300 g of water and tested as an aluminum cleaner.

Results of these observations and tests were as follows:

| Example | Silicon-based Material                                              | Acid Compatibility | Cleanability                                                  |
|---------|---------------------------------------------------------------------|--------------------|---------------------------------------------------------------|
| 35      | gamma-amino Propyl trimethyl siloxane                               | Dispersion formed  | Composition turned black and can become clean during rinse    |
| 36      | gamma-methoxy-acryloxy Propyl trimethyl siloxane                    | Same as Example 35 | Same as Example 35                                            |
| 37      | gamma-methoxy-acryloxy Propyl trimethyl siloxane (different source) | Same as Example 35 | Same as Example 35                                            |
| 38      | organofunctional silane                                             | Clear solution     | Composition turned very black and can did not rinse clean     |
| 39      | organofunctional silane (different source)                          | Clear solution     | Composition turned slightly black and can did not rinse clean |
| 40      | gamma-mercaptop Propyl trimethyl siloxane                           | Dispersion formed  | Same as Example 39                                            |

-continued

| Example | Silicon-based Material                                     | Acid Compatibility                                                       | Cleanability       |
|---------|------------------------------------------------------------|--------------------------------------------------------------------------|--------------------|
| 41      | gamma-mercaptopropyl trimethyl siloxane (different source) | Clear solution                                                           | Very poor cleaning |
| 42      | N-beta-aminoethyl gamma-amino Propyl trimethyl siloxane    | Violent reaction-neutralization of amine and production of gummy residue | Not tried          |
| 43      | Acrylic modified silane                                    | Material solidified                                                      | Not tried          |

The results indicate that acid compatible, sulfur-free siloxane materials provide beneficial aluminum cleaning. In contrast, the silanes and the mercapto siloxanes, although acid compatible and possibly effective defoamers, do not provide such beneficial aluminum cleaning effects. Care is to be exercised to avoid siloxane materials which react, e.g., in an acid/base neutralization reaction, with the acid or acids present in the composition.

#### EXAMPLE 44

A concentrate was prepared by blending together the following components:

|                                         | Wt. % |
|-----------------------------------------|-------|
| Sulfactant XIII                         | 34.4  |
| Enzyme A                                | 8.5   |
| Lithium salt of fluoroalkylthionyl acid | 2.0   |
| Sulfactant IV                           | 6.1   |
| gamma-amino Propyl trimethyl siloxane   | 1.0   |
| Water                                   | 48.0  |

A composition was prepared by blending together 2 g of this concentrate, 23 g of the acid composition of Example 24 to 29 and 300 ml of water.

This composition is tested as an aluminum cleaner in accordance with the procedure outlined in Example 1, and is found to provide excellent aluminum cleaning.

#### EXAMPLES 45 AND 46

Two samples of the composition of Example 44 were prepared for testing. One of the samples included 100 ppm (by weight) of fluoride ion.

The composition samples were tested as follows:

Two pieces of aluminum were dipped in concentrated chlorine-based bleach solution overnight. A black, smutty material became etched on these aluminum pieces as a result of this dipping.

One piece of aluminum was immersed in the composition sample without added fluoride ion at 130° F. for 10 minutes. The black smut was completely removed.

The other piece of aluminum was immersed in the composition sample with the added fluoride at 130° F. for 7 minutes. Not only was the black smut completely removed, but also the aluminum piece became bright and shiny.

These results indicate that the present compositions can be used to clean up aluminum that has been etched in a caustic solution. The addition of fluoride ion, preferably at low concentrations in the range of about 1 ppm to about 500 ppm by weight, enhances the aluminum cleaning action of the present corporation.

15 While this invention has been described with respect to various specific examples and embodiments, it is to be understood that the invention is not limited thereto and that it can be variously practiced within the scope of the following claims.

#### WHAT IS CLAIMED IS:

1. A composition useful for cleaning debris from an aluminum-containing article comprising: water; at least one polycarboxylic acid component selected from the group consisting of polycarboxylic acids, salts of polycarboxylic acids and mixtures thereof; at least one acidic component in an amount effective to increase the solubility of said polycarboxylic acid component in said composition; and at least one acid acting enzyme in an amount effective to at least facilitate the removal of debris from an aluminum-containing article contacted with said composition.

2. The composition of claim 1 wherein said polycarboxylic acid component is present in an amount effective to at least facilitate at least one of the following: (1) 20 remove at least a portion of said debris from said aluminum-containing article; and (2) condition at least a portion of said debris for removal from said aluminum-containing article.

3. The composition of claim 1 wherein said polycarboxylic acid component is selected from the group consisting of racemic tartaric acid, salts of racemic tartaric acid and mixtures thereof.

4. The composition of claim 1 wherein said acidic component is selected from the group consisting of sulfuric acid, phosphoric acid and mixtures thereof.

5. The composition of claim 4 which further comprises about 1 ppm to about 500 ppm by weight of fluoride ion.

6. The composition of claim 1 which further comprises at least one surface active component selected from the group consisting of nonionic surfactants, anionic surfactants and mixtures thereof.

7. The composition of claim 1 which further comprises at least one acid compatible, siloxane component in an amount effective to at least facilitate the removal of at least a portion of said debris from said aluminum-containing article.

8. The composition of claim 7 wherein said acid compatible, siloxane component is substantially sulfur free.

9. A composition useful for cleaning debris from an aluminum-containing article comprising: water; at least one polycarboxylic acid component selected from the group consisting of polycarboxylic acids, salts of polycarboxylic acids and mixtures thereof; at least one acidic component in an amount effective to increase the solubility of said polycarboxylic acid component in said composition; and at least one acid compatible, siloxane component in an amount effective to at least facilitate

the removal of at least a portion of said debris from said aluminum-containing article.

10. The composition of claim 9 wherein said acid compatible, siloxane component is substantially sulfur free.

11. The composition of claim 9 wherein said polycarboxylic acid component is present in an amount effective to at least facilitate at least one of the following: (1) remove at least a portion of said debris from said aluminum-containing article; and (2) condition at least a portion of said debris for removal from said aluminum-containing article.

12. The composition of claim 9 wherein said polycarboxylic acid component is selected from the group consisting of racemic tartaric acid, salts of racemic tartaric acid and mixtures thereof.

13. The composition of claim 9 wherein said acidic component is selected from the group consisting of sulfuric acid, phosphoric acid and mixtures thereof.

14. The composition of claim 13 which further comprises about 1 ppm to about 500 ppm by weight of fluoride ion.

15. The composition of claim 9 which further comprises at least one surface active component selected from the group consisting of nonionic surfactants, anionic surfactants and mixtures thereof.

16. A process for cleaning debris from the surface of an aluminum-containing article comprising:

contacting a debris-laden aluminum containing article with a composition at conditions effective to do at least one of the following: (1) remove at least a portion of said debris from said aluminum-containing article and (2) condition at least a portion of said debris for removal from said aluminum containing article, said composition comprising water; at least one polycarboxylic acid component selected from the group consisting of polycarboxylic acids, salts of polycarboxylic acids and mixtures thereof; at least one acidic component in an amount effective to increase the solubility of said polycarboxylic acid component in said composition; and at least one acid acting enzyme in an amount effective to at least facilitate the removal of debris from said aluminum-containing article; and

10

15

20

25

35

40

45

recovering said aluminum-containing article having at least a portion of said debris removed therefrom.

17. The process of claim 16 wherein said polycarboxylic acid component is present in an amount effective to at least facilitate at least one of the following: (1) remove at least a portion of said debris from said aluminum-containing article; and (2) condition at least a portion of said debris for removal from said aluminum-containing article.

18. The process of claim 16 wherein said polycarboxylic acid component is selected from the group consisting of racemic tartaric acid, salts of racemic tartaric acid and mixtures thereof.

19. The process of claim 16 wherein said composition further comprises at least one acid compatible, siloxane component in an amount effective to at least facilitate the removal of at least a portion of said debris from said aluminum-containing article.

20. A process for cleaning debris from the surface of an aluminum-containing article comprising:

contacting a debris-laden aluminum containing article with a composition at conditions effective to do at least one of the following: (1) remove at least a portion of said debris from said aluminum-containing article and (2) condition at least a portion of said debris for removal from said aluminum containing article, said composition comprising water; at least one polycarboxylic acid component selected from the group consisting of polycarboxylic acids, salts of polycarboxylic acids and mixtures thereof; at least one acidic component in an amount effective to increase the solubility of said polycarboxylic acid component in said composition; and at least one acid compatible, siloxane component in an amount effective to at least facilitate the removal of at least a portion of said debris from said aluminum-containing article.

21. The process of claim 20 wherein said acid compatible, siloxane component is substantially sulfur free.

22. The process of claim 20 wherein said polycarboxylic acid component is selected from the group consisting of racemic tartaric acid, salts of racemic tartaric acid and mixtures thereof.

\* \* \* \* \*

50

55

60

65

UNITED STATES PATENT AND TRADEMARK OFFICE  
CERTIFICATE OF CORRECTION

PATENT NO. : 4,959,105

Page 1 of 2

DATED : September 25, 1990

INVENTOR(S) : Fred Neidiffer et al

It is certified that error appears in the above-identified patent and that said Letters Patent is hereby corrected as shown below:

Column 8, line 13 change "has prepared" to -- was prepared --.

Column 9, line 66 through column 10, line 9 delete  
"As a base line, the ...e.g., beverage cans."

Column 10, line 35 and column 10, line 40 after the  
second occurrence of "Example" insert -- 15 --.

Column 11, line 10 change "as prepared" to -- was prepared --.

Column 12, lines 30-35 delete "While this invention...following  
claims."

Column 16, line 35 change "remove" to -- the removal of --.

Column 16, line 36 change "condition" to -- the conditioning of --.

Column 16, line 41 delete "racemic" each occurrence.

Column 17 line 15 delete "racemic" each occurrence.

Column 18, lines 5-6 change "remove" to -- the removal of --.

Column 18, line 7 change "condition" to -- the conditioning of --.

Column 18, line 12 delete "racemic" each occurrence.

Column 18, line 42 delete "racemic" each occurrence.

UNITED STATES PATENT AND TRADEMARK OFFICE  
CERTIFICATE OF CORRECTION

PATENT NO. : 4,959,105

Page 2 of 2

DATED : September 25, 1990

INVENTOR(S) : Fred Neidiffer, et al.

It is certified that error appears in the above-identified patent and that said Letters Patent is hereby corrected as shown below:

Title page:

Item (54) and column 1, in the title, change  
"ALUMINIUM" to --ALUMINUM--.

Signed and Sealed this  
Eighteenth Day of August, 1992

*Attest:*

DOUGLAS B. COMER

*Attesting Officer*

*Acting Commissioner of Patents and Trademarks*